

1,198,962.

I. ROSENBLUM.  
ELECTRICAL PROTECTIVE DEVICE.  
APPLICATION FILED OCT. 19, 1914.

Patented Sept. 19, 1916.

Fig. 1.



Fig. 2.



Fig. 3.



Witnesses:

Carl G. Yellock.  
J. Ellis Elam.

Inventor:  
Israel Rosenblum,  
by Almond, Davis  
His Attorney.

# UNITED STATES PATENT OFFICE.

ISRAEL ROSENBLUM, OF LYNN, MASSACHUSETTS, ASSIGNEE TO GENERAL ELECTRIC COMPANY, A CORPORATION OF NEW YORK.

## ELECTRICAL PROTECTIVE DEVICE.

1,198,962.

Specification of Letters Patent. Patented Sept. 19, 1916.

Application filed October 19, 1914. Serial No. 867,328.

To all whom it may concern:

Be it known that I, ISRAEL ROSENBLUM, a subject of the King of Roumania, residing at Lynn, in the county of Essex, State of Massachusetts, have invented certain new and useful Improvements in Electrical Protective Devices, of which the following is a specification.

10 The present invention comprises a resistance unit of simple and rugged construction having breaking down at a critical voltage which may be fixed at will for a given unit, and suitable particularly as a cutout or protective device or for other purposes.

15 It is the object of my invention to produce a unit of this character which can be given in its manufacture the particular electrical properties adapting it for the purpose intended, and which after repeated 20 operation will retain substantially the same characteristics.

While my invention has particular reference to the utilization of boron in electrical cut-out devices, the principle of its construction is likewise applicable to similar substances, such, for example, as silicon.

In accordance with one feature of my invention I have provided a cut-out in which a film of boron is united to a material of 30 relatively high conductivity, such, for example, as carbon. An intimate union is produced by chemically depositing at high temperature a film of boron on a conductor of carbon, boro-carbon, tungsten, or the like, 35 and by depositing in turn upon the boron a layer of one of these good conducting materials, thereby producing a unitary structure.

Another feature of my invention is a cut-out, the breakdown voltage of which may be accurately adjusted during manufacture to any desired voltage range.

In the accompanying drawings Figure 1 shows in section a simple form of boron cut-out greatly magnified; Fig. 2 is a modification in which two layers of boron are, interposed in the electrical circuit, and Fig. 3 is a sectional view of a boron-cut-out mounted in an envelop and provided with terminals

suitable for convenient insertion into clips or similar contact-making devices.

Boron because of its high electrical resistance and very high negative temperature coefficient of resistance is peculiarly adapted to use as an electrical cut-out material, but 5 the very great hardness, crystalline and brittle character of boron and its oxidizability render the construction of such a cut-out extremely difficult. This will be readily seen when it is borne in mind that the high 60 resistance of boron makes it necessary to use a thin layer in cut-outs designed to be operated at a moderate voltage, and that contacts must be provided which will not necessarily raise the resistance of the unit and 65 will not vary in resistance when heated by a passage of current.

Because of the physical properties of boron difficulties are experienced with the maintenance of the electrical contacts. Mechanical 70 contacts and soldered contacts have proved to be not reliable.

My cut-out preferably takes the form of a rod-like body, as shown greatly magnified in Fig. 1. The core 1 consists of conductive material, preferably of boro-carbon. The boro-carbon may be prepared by squirting finely divided boron with pitch and carbonizing the product, the amount of pitch introduced being varied in accordance with 75 the break-down voltage desired. Tungsten or other refractory metal may be added to increase the conductivity of the core. Upon the core is deposited a layer of boron 2 by heating the core in a mixture of boric chloride and hydrogen, as described in U. S. Patent #1,019,393 to E. Weintraub. Mechanical shaping of the brittle boron is thus avoided and an intimate adherence is secured which, being free from soldering material, and being formed by the deposition 80 of the boron molecules as they are set free from a compound in the gaseous state may be called a molecular union. The thickness 85 of the layer depends on the length of time 90 that deposition at incandescence is continued, and also on the temperature and proportions 95 of the treating mixture. The break-down

voltage of boron is best adjusted by introducing a very small but definite quantity of carbon. The above Weintraub Patent #1,019,393 discloses a method of adding carbon to boron by depositing the boron and carbon simultaneously from a mixture of boric chlorid and hydrocarbon, but because the amounts of carbon required in the boron layer of a cut-out are extremely minute, this method ordinarily is not refined enough.

I have found that by using a base filament of boro-carbon and depositing boron on this base enough carbon may be transferred from the base to the deposited boron to give the necessary adjustment of breakdown voltage. By increasing the amount of carbon in the base greater amounts of carbon may be transferred to the boron layer.

The conductor thus prepared is then 20 candesced in a hydrocarbon atmosphere, such as a vapor of benzol; gasolene, carbon tetrachlorid, or the like, until a layer 3 of carbon of suitable thickness has been deposited. Here again an intimate molecular 25 adherence of the carbon to the boron is secured and an electrical contact is provided which is unaffected by thermal changes.

If but a single layer of boron is to be included in the electrical circuit the end of the 30 core 1 may be exposed by grinding off part of the deposited layers, the carbon being removed from all except the end, as shown in Fig. 1. If, on the other hand the breakdown of two layers of boron is desired, the 35 layer of boron and the films of carbon 3, 4 may be allowed to remain at each of the end portions as shown in Fig. 2. As shown in Fig. 3, a unit thus constructed may be provided with terminal sleeves 5, 6, preferably 40 consisting of graphite, and simply making a mechanically tight fit with the deposited layer of carbon. A unit thus made is slipped into a protective sheath 7 of glass or other non-conducting material and provided with 45 metallic end caps 8, 9, which may have conductive stems 10, 11 centering and holding the graphite sleeves. When a unit thus constructed is connected in shunt with a device, such as a series connected arc lamp or incandescent lamp, and the voltage across its 50 terminals rises above the value at which the boron layer has been proportioned to break down in resistance, an electrical circuit is established from the layer of carbon 3 through the layer of boron to the core 1, to 55 which contact may be made in the simple form of cut-out shown in Fig. 1, or from the core through another layer of boron to the second layer of carbon, as shown in Figs. 60 2 and 3.

Cut-outs as above described may be made to break down at any commercial voltage, for example, from 500 volts down and will

be substantially invariable in their breakdown characteristic between successive periods of operation. The voltage range within which the cut-out may be constructed to break down can be adjusted not only by varying the thickness of the boron film, the temperature, the concentration of boron vapors and other factors during the treatment and the percentage of carbon in the boro-carbon base, as above indicated, but also by varying the surface of the contact between the carbon or other conductive terminal and the boron, and the degree of heat dissipation effected by the terminals. As pointed out in Thomson Patent No. 1,063,303, an increase in the size of the heat radiating members in contact with the boron increases the voltage and lengthens the time necessary for causing the breakdown of the boron film. It is, therefore, difficult to give any specific example, but it will be obvious by varying any or all of these means of adjustment cut-outs may be constructed for any desired service.

What I claim as new and desire to secure by Letters Patent of the United States, is:—

1. An electrical cut-out comprising a film-like body of extended surface consisting largely of boron and bodies of highly conductive material molecularly adhering to opposite surfaces of said boron body to form a unitary structure. 95
2. An electrical cut-out comprising a film-like body of extended surface consisting largely of boron and bodies of carbon molecularly united therewith. 100
3. An electrical cut-out comprising a film of boron associated with carbon, and bodies of highly conductive material molecularly adhering thereto. 105
4. An electrical cut-out comprising a core of conductive material, a layer consisting largely of boron molecularly united thereto, and a layer of carbon molecularly united with said boron layer. 110
5. An electrical cut-out comprising a rod of boro-carbon, a relatively thin layer of boron deposited thereon and adhering intimately thereto, a layer of carbon deposited on said boron and adhering thereto, and conductors contacting respectively with said rod and carbon layer. 115
6. An electrical cut-out comprising a rod-like body consisting of boron and carbon, a layer of boron united with said body, layers of carbon covering the end portions only of said boron layer and intimately united therewith, sleeves of graphite mechanically inclosing said carbon layers and making electrical contact therewith. 120
7. An electrical cut-out consisting of a rod-like body of boro-carbon, and a layer of boron molecularly united therewith, layers

of carbon intimately united with the end portions of said boron layer, graphite sleeves mechanically fitted to said carbon layers at each end of said body, and current-carrying terminals for said graphite sleeves.

8. An electrical cut-out comprising a core of boro-carbon, a film consisting largely of boron molecularly united thereto and a

layer of carbon molecularly united with said boron layer.

In witness whereof, I have hereunto set my hand this fifteenth day of October, 1914.

ISRAEL ROSENBLUM.

Witnesses:

JOHN A. McMANUS, JR.,  
JOHN T. BEECILYN.